

## UNITED STATES PATENT OFFICE

2,648,628

## ELECTROPLATING OF NICKEL

Henry Brown, Detroit, Mich., assignor to The  
Udylite Corporation, Detroit, Mich., a corpora-  
tion of Delaware

No Drawing. Application July 17, 1950,  
Serial No. 174,375

12 Claims. (Cl. 204—49)

1

My invention relates to improvements in the electro-deposition of nickel from aqueous acidic baths. It is particularly concerned with the utilization of mixtures of certain types of agents for the purpose of decreasing grain size and increasing the luster of the nickel plate or deposit, and it is especially concerned with the production of electrodeposits of brilliant, highly lustrous, ductile nickel plates.

I have discovered that the above highly desired results are achieved through the conjoint utilization, in the nickel plating bath, of one or more agents of the type exemplified in the following Table I, in conjunction with one or more agents of the type exemplified in the following Table II.

The agents of Table I are illustrative of the class of compounds, found to be useful in the practice of my present invention, in accordance with the formula



where



represents a compound selected from the group consisting of quinoline, isoquinoline and C-methyl and ethyl homologues thereof; R is halogen, such as chlorine, bromine or iodine, particularly chlorine and bromine; and x is zero to 2. These compounds can be and preferably are used in the form of salts thereof, e. g. the hydrochlorides, sulfates, and formates, and when reference is made to said compounds hereafter and in the claims, it will be understood to encompass both the free bases and the acid salts thereof.

As indicated, R is halogen and, as x can be zero, 1 or 2, the compounds can contain one or two nuclear halogen groups or, where x is zero, the nucleus is unsubstituted. Excellent results are obtained with compounds where x is zero;

or where R is chlorine or bromine and x is 1. Of outstanding utility are 2-methyl quinoline and 3-methyl isoquinoline. Good results are also obtained with quinoline, isoquinoline, and 2,6-dimethyl quinoline or mixtures of any two or more thereof, or mixtures of 2-methyl quinoline with one or more of the other compounds disclosed herein. It will be understood, of course, that pure or commercial sources of said compounds can be employed and, in general, commercial sources of certain of said compounds will usually be found to contain minor proportions of others of said compounds. Thus, for example, commercial 2-methyl quinoline ordinarily contains about 5% isoquinoline.

2

TABLE I

|    |                                 | Quinoline and Isoquinoline Compounds | Optimum Conc., Grams/liter |
|----|---------------------------------|--------------------------------------|----------------------------|
| 20 | 1. Quinoline                    | .005-.02                             |                            |
|    | 2. Isoquinoline                 | .003-.02                             |                            |
|    | 3. 2-methyl quinoline           | .005-.03                             |                            |
|    | 4. 8-iodo quinoline             | .005-.03                             |                            |
|    | 5. 2,6-dimethyl quinoline       | .005-.03                             |                            |
|    | 6. 2-chloro quinoline           | .005-.03                             |                            |
|    | 7. 6-bromo quinoline            | .005-.03                             |                            |
|    | 8. 3-methyl quinoline           | .005-.03                             |                            |
|    | 9. 2,4,6-trimethyl quinoline    | .005-.03                             |                            |
|    | 10. 2-ethyl quinoline           | .005-.02                             |                            |
|    | 11. 2-bromo quinoline           | .005-.03                             |                            |
|    | 12. 6-bromo isoquinoline        | .003-.02                             |                            |
|    | 13. 6-methyl isoquinoline       | .003-.03                             |                            |
|    | 14. 2,4-dibromo quinoline       | .005-.03                             |                            |
|    | 15. 2,4-dichloro quinoline      | .005-.03                             |                            |
|    | 16. 2,8-dimethyl quinoline      | .003-.02                             |                            |
|    | 17. 1,3-dimethyl isoquinoline   | .003-.03                             |                            |
|    | 18. 3-methyl isoquinoline       | .005-.03                             |                            |
|    | 19. 2-methyl-8-bromo quinoline  | .005-.03                             |                            |
| 35 | 20. 2-methyl-8-chloro quinoline | .005-.03                             |                            |
|    | 21. 3-chloro-2-methyl quinoline | .005-.03                             |                            |
|    | 22. 3-bromo-2-methyl quinoline  | .005-.03                             |                            |
|    | 23. 1-methyl isoquinoline       | .003-.03                             |                            |

40

The agents of Table II are illustrative of the class of compounds which are employed in conjunction with the agents of Table I, in the practice of my invention. The agents of Table II, it will be noted, fall into the category of organic sulfonamides, sulfonimides and sulfonic acids. They have heretofore been used as brighteners in nickel plating baths as is disclosed in part, for example, in my prior Patents Nos. 2,191,813

and 2,466,677. In the practice of my present invention, a coaction takes place in the cathode film, the exact nature of which is unknown, involving the compounds of the type shown in Table I and the organic sulfur-containing brightener which produces the unusual and highly important results which are brought about in accordance with my invention. In this connection, it may be noted that the utilization alone of the agents or compounds of the type shown in Table I, or the utilization alone of the organic sulfur-containing brighteners, gives no indication of the remarkably enhanced results which occur when both types of compounds are present in the bath, particularly when utilized in their optimum concentrations. In general, it is desirable to use mixtures of two or more of said sulfur-containing brighteners as, for example, o-benzoyl sulfimide and p-toluene sulfonamide; and allyl sulfonic acid and benzene sulfonamide.

TABLE II

| Sulfur-Containing Brighteners                      | Optimum Conc., Grams/liter |
|----------------------------------------------------|----------------------------|
| 1. Benzene sulfonamide                             | 0.1-3                      |
| 2. Toluene sulfonamides (o and p)                  | 0.1-2                      |
| 3. o-Benzoyl sulfimide                             | 0.1-2                      |
| 4. N-Benzoyl benzene sulfonimide                   | 0.1-1                      |
| 5. p-Toluene sulfonchloramide                      | 0.1-1                      |
| 6. p-Brom benzene sulfonamide                      | 0.1-1                      |
| 7. 6-Chlor o-benzoyl sulfimide                     | 0.1-1                      |
| 8. m-Aldehydo benzene sulfonamide                  | 0.1-1                      |
| 9. Sulfomethyl benzene sulfonamide                 | 0.1-6                      |
| 10. Benzene sulfonamide m-carboxylic amide         | 0.1-3                      |
| 11. 7-Aldehydo o-benzoyl sulfimide                 | 0.1-3                      |
| 12. N-Acetyl benzene sulfonimide                   | 0.1-2                      |
| 13. Methoxy benzene sulfonamides                   | 0.1-1                      |
| 14. Hydroxymethyl benzene sulfonamide              | 0.1-2                      |
| 15. Vinyl sulfonamide                              | 4-12                       |
| 16. Allyl sulfonamide                              | 4-12                       |
| 17. Benzene sulfonic acids (mono, di, and tri)     | 1-15                       |
| 18. p-Brom benzene sulfonic acid                   | 3-6                        |
| 19. Benzaldehyde sulfonic acids (o, m, p)          | 2-6                        |
| 20. Diphenyl sulfone sulfonic acid                 | 1-8                        |
| 21. Naphthalene sulfonic acids (mono, di, and tri) | 1-8                        |
| 22. Benzene sulfohydroxamic acid                   | 1-5                        |
| 23. p-Chlor benzene sulfonic acid                  | 1-15                       |
| 24. Diphenyl sulfonic acid                         | 1-5                        |
| 25. m-Diphenyl benzene sulfonic acid               | 1-4                        |
| 26. 2-Chloro-5-sulfobenzaldehyde                   | 1-5                        |
| 27. m-Benzene disulfonamide                        | 0.5-1                      |
| 28. Allyl sulfonic acid                            | 4-12                       |

It will be understood that said sulfonic brighteners may be utilized in their acid form or in the form of salts as, for example, nickel, sodium, potassium or other salts. Especially satisfactory, for use in the practice of my present invention, are the compounds of Table II corresponding to numbers 1, 2, 3; 18, 19, 21 and 28, the latter particularly in the form of their nickel salts. Where the term sulfonic acids is used herein and in the claims, it will be understood that the salts thereof are likewise included.

The compounds of Table II, used alone, produce reasonably bright deposits on buffed metals such as buffed brass. However, at least in the ordinary case, they do not accomplish the same results on steel polished with 180 emery or on matte (but unburnt) copper plate of 0.0003"-0.0005" thickness but, rather, generally yield plates of somewhat dull and gray appearance in these cases. The compounds of Table I, in the usual case, when used alone, give a different type of plate than that produced by the compounds of Table II. The plates produced with the compounds of Table I alone are fine grained and cloudy at very low concentrations, and are rather

dark, brittle, easily stained and have poor adherence characteristics at higher concentrations. If, however, the two different types of compounds represented in Tables I and II are used together in the baths, as I have indicated above, brilliant mirror-like, adherent and ductile deposits are obtained even over matte surfaces.

Only small proportions of the compounds, or mixtures thereof, of Table I are necessary to achieve the aforesaid results. Generally, proportions in the range of about 0.003 gram/liter to about 0.04 gram/liter of any of the compounds or mixtures thereof will be most effective in the usual case although, particularly with the more efficacious ones of the compounds, proportions even as low as about 0.001 gram/liter give good results. Even in the case of the less effective ones of the compounds, it is rarely necessary to exceed about 0.04 gram/liter. As a general rule, the optimum concentration of the compounds will be found to fall within the range of about 0.005 to about 0.03 gram/liter.

The compounds of Table II are likewise used in small proportions, in conjunction with the compounds of Table I, amounts of the order of about 0.1 gram/liter to 2 or 3 grams/liter being effective in the usual case. Higher proportions, up to saturation, can, however, be utilized. Ordinarily, it is unnecessary to exceed about 0.5%.

The optimum concentration of the compounds of Tables I and II in any specific instance may readily be determined by simple test in the light of the particular nickel bath utilized, its temperature, its pH, etc.

The aqueous nickel plating baths may be of various types but, in all cases, they are acidic in character. The preferred baths are of the so-called acidic "grey" type which are capable of producing thick, adherent, ductile deposits, those of the Watts type or modifications thereof being particularly desirable. The nickel salts may comprise nickel chloride, nickel sulfate, nickel fluoborate, nickel sulfamate, or other nickel salts or mixtures of any two or more of said nickel salts, preferably in conjunction with buffer materials as, for example, boric acid. I prefer to utilize boric acid in the bath as it is, in general, the best cathode film buffer. Other buffers of acidic character may, however, be employed as, for example, formic acid, citric acid, fluoboric acid, and the like, and such may be used either in place of or in conjunction with boric acid. For optimum results, the concentration of the boric acid or its equivalent should be above 30 grams per liter, especially in baths operated at somewhat elevated temperatures. The baths may also contain various supplemental agents such as anti-pitting agents and the like.

The baths can be operated at temperatures ranging from about room temperature to almost boiling but, in general, the preferred temperature is in the range of about 40 degrees C. to 65 degrees C. In general, the baths can be operated at pH values ranging from about 2 to about 5.5 but, in the ordinary case, the preferred pH values are from 2.5 to 4.8. The cathode current density ranges are quite variable, a range of about 5 to several hundred amperes per square foot being utilizable, the optimum depending upon agitation, temperature, and concentration and type of nickel salts utilized in the bath. A good working range is about 20 to about 80 amperes per square foot. In Table III, I list preferred embodiments of bath compositions.

TABLE III

| Bath No. | $\text{NiSO}_4 \cdot 6\text{H}_2\text{O}$ , Grams/liter | $\text{NiCl}_2 \cdot 6\text{H}_2\text{O}$ , Grams/liter | $\text{Ni}(\text{BF}_4)_2$ , Grams/liter | $\text{H}_3\text{BO}_3$ , Grams/liter | Temperature, °F. | pH         | Current Density, Amps/sq.ft. | Addition Agents, grams/liter                                                                                                           |
|----------|---------------------------------------------------------|---------------------------------------------------------|------------------------------------------|---------------------------------------|------------------|------------|------------------------------|----------------------------------------------------------------------------------------------------------------------------------------|
| 1        | 200 to 300                                              | 45                                                      |                                          | 40                                    | 75 to 160        | 2 to 6     | 10 to 75                     | {2-methyl quinoline—.005 to .03.<br>o-benzoyl sulfimide—1.<br>2-methyl quinoline—.003 to .02.<br>Quinoline—.003.                       |
| 2        |                                                         | 300                                                     |                                          | 40                                    | 75 to 160        | 1 to 5     | 10 to 100                    | Benzene sulfonamide—2.<br>o-benzoyl sulfimide—2.<br>8-methyl quinoline—.015.<br>p-toluene sulfonamide—1.5.<br>o-benzoyl sulfimide—0.1. |
| 3        | 50 to 200                                               | 100 to 250                                              |                                          | 40                                    | 75 to 160        | 1.5 to 6   | 10 to 85                     | 2-chloro quinoline—.006 to .02.<br>Benzene sulfonamide—2.<br>2-bromo isoquinoline—.004 to .02.                                         |
| 4        | 200 to 300                                              | 45 to 75                                                | 4 to 8                                   | 40 to 50                              | 75 to 160        | 2 to 6     | 10 to 75                     | o-benzoyl sulfimide—2.<br>o-benzoyl sulfimide—1.                                                                                       |
| 5        | 200 to 300                                              | 45 to 100                                               | 8 to 50                                  | 40 to sat                             | 75 to 160        | 2 to 6     | 10 to 85                     | 2-methyl isoquinoline—.004 to .02.<br>o-benzoyl sulfimide—2.<br>2-methyl quinoline—.005 to .03.                                        |
| 6        | 50 to 100                                               | 45 to 100                                               | 8 to 100                                 | 40 to sat                             | 75 to 160        | 2 to 6     | 10 to 85                     | o-benzoyl sulfimide—1.<br>p-toluene sulfonamide—1.<br>3-methyl isoquinoline—.003 to .02.<br>o-benzoyl sulfimide—1.                     |
| 7        |                                                         | 45 to 100                                               |                                          | 50 to 150                             | 40 to sat        | 75 to 160  | 2 to 6                       | Benzene sulfonamide—1.<br>2-methyl quinoline—.003.<br>Quinoline—.002.                                                                  |
| 8        | 200 to 250                                              | 100 to 150                                              | 8 to 15                                  | 40 to 50                              | 75 to 160        | 2 to 6     | 10 to 85                     | o-Benzaldehyde sulfonic acid—3 to 8.<br>2,4-dimethyl quinoline—.008 to .02.                                                            |
| 9        |                                                         |                                                         |                                          | 100 to 300                            | 0 to sat         | 75 to 160  | 4 to 5                       | Naphthalene sulfonic acids—3 to 6.<br>Quinoline—.006 to .02.                                                                           |
| 10       | 200 to 300                                              | 100 to 75                                               |                                          | 40                                    | 110 to 140       | 3 to 4.5   | 40 to 60                     | Allyl sulfonic acid—6.<br>2,6-dimethyl quinoline—.02.                                                                                  |
| 11       | 100 to 200                                              | 200 to 100                                              |                                          | 40                                    | 110 to 140       | 3 to 4.5   | 40 to 60                     | o-benzoyl sulfimide—1.<br>p-toluene sulfonamide—1.<br>Quinoline—.005 to .015.                                                          |
| 12       | 300                                                     | 60                                                      |                                          | 40                                    | 70 to 160        | 2.5 to 4.8 | 40 to 60                     | 2-methyl quinoline—.005 to .015.<br>p-toluene sulfonamide—1 to 2.<br>o-benzoyl sulfimide—1 to 3.<br>Isoquinoline—.006.                 |
| 13       | 225                                                     | 50 to 75                                                |                                          | 40                                    | 70 to 160        | 2.5 to 4.8 | 40 to 60                     | 2-methyl quinoline—.015.<br>Benzene sulfonamide—2.<br>o-benzoyl sulfimide—2.                                                           |

It will be understood that, from time to time, it is necessary to replenish the bath to replace losses due to cathodic processes, to "drag-out," and to other causes, in order to maintain the concentrations of the added compounds, etc. in operative proportions.

This application is a continuation-in-part of my application Serial No. 587,427, filed April 9, 1945, said latter application being, in turn, a continuation-in-part of my application Serial No. 366,386, filed November 20, 1940, all of said applications being now abandoned.

What I claim as new and desire to protect by Letters Patent of the United States is:

1. A bath for the electrodeposition of bright nickel comprising an aqueous acidic solution containing at least one nickel salt selected from the group consisting of nickel chloride and nickel sulfate, said bath also containing, in solution, not more than 15 grams per liter of at least one brightener selected from the group consisting of organic sulfonamides, sulfonimides, and sulfonic acids, and, in addition, from about 0.005 to about 0.04 gram per liter of a bath-soluble compound in accordance with the formula



where



represents a compound selected from the group consisting of quinoline, isoquinoline and C-methyl and ethyl homologues thereof, R is halogen, and x is zero to 2.

2. A bath for the electrodeposition of bright nickel comprising an aqueous acidic solution of at least one nickel salt, said bath also containing, in solution, not more than about 15 grams

per liter of at least one brightener selected from the group consisting of organic sulfonamides, sulfonimides, and sulfonic acids, and, in addition, .005—.04 gram per liter of 2-methyl quinoline.

3. A bath for the electrodeposition of bright nickel comprising an aqueous acidic solution containing at least one nickel salt selected from the group consisting of nickel chloride and nickel sulfate, said bath also containing, in solution, not more than about 15 grams per liter of at least one brightener selected from the group consisting of organic sulfonamides, sulfonimides, and sulfonic acids, and, in addition, from about 0.005 to about 0.04 gram per liter of 2-methyl quinoline.

4. A bath for the electrodeposition of bright nickel comprising an aqueous acidic solution containing at least one nickel salt selected from the group consisting of nickel chloride, and nickel sulfate, said bath also containing, in solution, not more than about 15 grams per liter of at least one brightener selected from the group consisting of organic sulfonamides, sulfonimides, and sulfonic acids, and, in addition, from about 0.005 to about 0.04 gram per liter of a bath-soluble compound in accordance with the formula



where R is a halogen selected from the group consisting of chlorine and bromine, and x is zero to 2.

5. A bath for the electrodeposition of bright nickel comprising an aqueous acidic solution containing at least one nickel salt selected from the group consisting of nickel chloride and nickel sulfate, said bath also containing, in solution, not more than about 0.5% of at least one brightener selected from the group consisting of organic sulfonamides, sulfonimides, and sulfonic acids, and, in addition, from about 0.005 to about

0.04 gram per liter of a mixture of isoquinoline and 2-methyl quinoline.

6. A bath in accordance with claim 1, wherein the compound



is isoquinoline.

7. A bath in accordance with claim 1, wherein the compound



is a C-methyl quinoline.

8. A method of electrodepositing nickel to obtain a fine-grained, ductile deposit of high brilliance which comprises electrolyzing an aqueous acidic solution containing at least one nickel salt selected from the group consisting of nickel chloride and nickel sulfate, said bath also containing, in solution, not more than about 15 grams per liter of at least one brightener selected from the group consisting of organic sulfonamides, sulfonimides, and sulfonic acids, and, in addition, from about 0.005 to about 0.04 gram per liter of a bath-soluble compound in accordance with the formula



where



represents a compound selected from the group consisting of quinoline, isoquinoline and C-methyl and ethyl homologues thereof, R is halogen, and x is zero to 2.

9. A method of electrodepositing nickel to obtain a fine-grained, ductile deposit of high brilliance which comprises electrolyzing an aqueous acidic solution of at least one nickel salt, said bath also containing, in solution, not more than about 0.5% of at least one brightener selected from the group consisting of organic sulfonamides, sulfonimides, and sulfonic acids, and, in addition, from about 0.005 to about 0.04 gram per liter of 2-methyl quinoline.

10. A method of electrodepositing nickel to obtain a fine-grained, ductile deposit of high brilliance which comprises electrolyzing an aqueous acidic solution containing at least one nickel salt selected from the group consisting of nickel chloride and nickel sulfate, said bath also containing, in solution, not more than about .5% of at least one brightener selected from the group consisting of organic sulfonamides, sulfonimides, and sulfonic acids, and, in addition, .005-.04 gram per liter of a bath-soluble compound in accordance with the formula



where R is a halogen selected from the group consisting of chlorine and bromine, and x is zero to 2.

11. In a bath for the electrodeposition of bright nickel comprising an aqueous acidic solution containing at least one nickel salt selected from the group consisting of nickel chloride and nickel sulfate, an additive for use in an amount of about .005 to about .04 gram per liter in combination with at least one brightener selected from the group consisting of organic sulfonamides, sulfonimides and sulfonic acids in an amount of not more than about 15 grams per liter in said bath, said additive consisting of a compound having the formula



20 where



represents a compound selected from the group 25 consisting of quinoline, isoquinoline and C-methyl and ethyl homologues thereof, R is halogen, and x is zero to 2.

12. An additive for an aqueous acidic solution containing at least one nickel salt selected from 30 the group consisting of nickel chloride and nickel sulfate and at least one brightener selected from the group consisting of sulfonamides, sulfonimides and sulfonic acids in an amount of not more than about 15 grams per liter in combination 35 with said additive in an amount of about .005 to about .04 gram per liter, said additive consisting of a compound having the formula



40 where



represents a compound selected from the group 45 consisting of quinoline, isoquinoline and C-methyl and ethyl homologues thereof, R is halogen, and x is zero to 2.

HENRY BROWN.

References Cited in the file of this patent

UNITED STATES PATENTS

| Number    | Name        | Date          |
|-----------|-------------|---------------|
| 2,238,861 | Lind et al. | Apr. 15, 1941 |
| 2,315,802 | Lind et al. | Apr. 6, 1943  |

OTHER REFERENCES

- 60 Raub et al., Metal Finishing, August 1940, pp. 429-432.